

1

3,809,559  
LIQUID AMINE-TYPE DEVELOPER FOR  
DIAZOTYPE MATERIALS

Henry J. Neuman, Chicago, Ill., assignor to Addressograph-Multigraph Corporation, Mount Prospect, Ill.  
No Drawing. Continuation of abandoned application Ser. No. 128,541, Mar. 26, 1971. This application June 8, 1973, Ser. No. 368,169

Int. Cl. G03c 5/34

U.S. Cl. 96—49

10 Claims

ABSTRACT OF THE DISCLOSURE

A developer liquid containing as the active ingredients at least 20% by weight of morpholine, piperidine, lower alkyl morpholine, lower alkyl piperidine, or an organic amine of the formula:



wherein R, R' and X are hydrogen, lower alkyl or lower hydroxy alkyl and n is an integer from 2 to 4, inclusive, and containing a diluent which may be a polyhydric alcohol, a glycol ether or a monofunctional alcohol and a third component which is a carboxylic fatty acid having a carbon chain length of from 16 to 18 carbon atoms such as oleic, linoleic, linolenic, stearic or palmitic and is present in an amount ranging from 1% to 20% by weight.

This is a continuation of application Ser. No. 128,541 filed Mar. 26, 1971, now abandoned.

BACKGROUND OF THE INVENTION

This invention relates to liquid developers for developing two-component diazotype materials in which the active ingredient is an organic amine and more particularly developer liquid compositions which can be used under conditions where small amounts of the liquid are spread over the latent image bearing surface of a two-component diazotype material.

Diazotype reproduction processes in which a two-component diazotype material is developed by applying a small amount of a developer liquid, usually not exceeding three grams per square meter of the latent image bearing surface are described in U.S. Pat. 3,446,620, issued to Konrad Parker on May 27, 1969, and assigned to the same assignee as the instant invention. This known technique which produces a dry copy directly from a liquid developing step is accomplished by supplying controlled amounts of the concentrated developer solution, comprising an aliphatic amine, to a two-component diazotype material. The technique calls for providing a developing region through which is passed the exposed diazotype paper where the controlled small amount of liquid is applied directly to the latent diazo image bearing surface to effectively develop the azo-dye image and the prints emerge dry, odor-free and ready for use.

The controlled amounts of liquid refer to the application of quantities not in excess of three grams of developer per square meter of the image bearing surface and preferably in the range of from about 0.5 gram to 2 grams per square meter.

The method which is described in 3,446,620, may be carried out by a number of different types of apparatus specifically designed to apply the controlled amounts. One such apparatus is described in U.S. application Ser. No. 831,685, now U.S. Pat. 3,626,833, assigned to the same assignee as the instant invention. It will be appreciated that in the construction of such developing apparatus, the usual and known techniques of applying a liquid to a surface are not routinely accomplished and require special consideration.

2

SUMMARY OF THE INVENTION

In the circumstance that liquid developer is applied at the rate of 1 or 2 grams per square meter of the two-component diazotype material, it is necessary that at the developing region the liquid is uniformly and evenly applied so that the azo-dye image which results is of a uniform dye density. It has been found that great stress is imposed on such apparatus applying the small amounts of developer liquid which must be uniformly spread over the entire image-bearing surface area.

Apparatus equipped with applicator rollers whose surface has been specially prepared to carry a controlled amount of liquid and operate in conjunction with a squeegee or wiping device to further monitor the amount of liquid, tends to generate high frictional forces at the developing stage. The high frictional stresses at the point of development impose a stress on the drive mechanism for the apparatus, which in turn causes erratic movement of the drive rollers. There is a perceptible variation in speed. Thus, the paper to be developed is advanced through the developer in the same erratic fashion causing image striations and irregularities in the copy due to irregular liquid application.

It is a general object of this invention to provide an improved liquid developer composition for developing two-component diazotype materials which permits the application of very small quantities of said liquid to be spread uniformly and evenly over the surface of the diazotype material.

It is another object of this invention to provide an improved liquid developer composition for developing two-component diazotype materials which tends to alleviate the stresses imposed on such developing equipment under the conditions of applying less than 3 grams of said developer liquid to the latent image bearing surface of the diazotype material.

It is a specific object of this invention to provide an improved developer liquid composition for developing two-component diazotype materials employing a concentrated solution of an aliphatic amine, and a carboxylic fatty acid increasing the lubricity of the system to greatly enhance the uniformity and evenness of application.

The objectives recited above are achieved by a new composition for developer liquids which comprise from 20% to 80% by weight of an active alkaline component such as an aliphatic amine, a diluent comprised of a polyhydric alcohol, a glycol ether or a monofunctional alcohol; and a carboxylic fatty acid having from 16 to 18 carbon atoms in an amount ranging from 1% to 20% by weight.

DESCRIPTION OF THE PREFERRED  
EMBODIMENTS

55 The following description sets forth the details of the developer which will achieve the objects set forth in the summary of the invention.

The alkaline component of the developer may be a compound having the general formula:



60 where R<sub>1</sub>, R<sub>2</sub> and R<sub>3</sub> are members selected from the group consisting of alkyl, cycloalkyl, alkyl-aryl, alkylol, alkoxy, hydroxy-alkoxyalkyl and hydrogen, and



70 represents a heterocyclic ring such as morpholine and piperidine.

The preferred amines useful in this invention are those which come within the formula:



wherein R and R' are the same or different alkyl or hydroxyalkyl radicals or hydrogen, X is hydrogen, alkyl or hydroxyalkyl, and n is an integer from 2 to 4, inclusive.

The alkaline component may be diluted with a compound selected from the group consisting of a polyhydric alcohol, a glycol-ether, a monofunctional alcohol and water or admixtures thereof. The diluent may be present in amounts ranging from 17% to 60% by weight of the formulation, the preferred range being from 30% to 50%.

The following amines have been eminently successful in the practice of the method: monoethanolamine, isopropanolamine, 2-(2-aminoethoxy)ethanol, triethanolamine, diethanolamine, 2-amino-2-methyl-1-propanol, N-methyl-ethanolamine, dimethylethanolamine, hexylamine, cyclohexylamine. Other amines have demonstrated the ability to develop the diazo print such as beta hydroxyethyl trimethyl ammonium carbonate, N-aminoethylethanolamine, alkyl substituted morpholine and piperidine, but are somewhat less desirable because they have a detectable odor or they tend to adversely affect the dye shade.

The use of a diluent aids in the spreadability and wetting out of the developer across the area to which it is applied. The diluent also finds utility as a material which can be used to adjust the viscosity of the developer liquid so that it can easily be pumped and caused to flow through various conduits to bring it to the developing region. In addition, if the diluent has a greater volatility than the aliphatic amine, it will tend to evaporate from the surface having a drying effect on the thin layer.

The diluent may be comprised of a polyhydric alcohol selected from the following:

hexylene glycol  
diethylene glycol  
polyethylene glycol  
trimethylene glycol  
ethylene glycol  
propylene glycol  
dipropylene glycol  
glycerine

and glycol-ethers such as:

ethylene glycol monoethyl ether (Cellosolve)  
diethylene glycol monoethyl ether  
diethylene glycol monomethyl ether  
butyl Cellosolve

or a monofunctional alcohol such as:

4-methoxy-4 methyl-pentanol-2(pentoxyl)  
2-ethyl hexanol  
cyclohexanol  
isooctyl alcohol  
hexanol

It has been found advantageous to use the polyhydric alcohols which are completely compatible with the aliphatic amines and do not adversely affect the print quality. Also, polyhydric alcohols such as, for example, hexylene glycol and glycol ethers enhance the spreadability of the developer liquid.

The advancement of this invention is represented by the addition of a third component such as a carboxylic fatty acid having a carbon chain length of from 16 to 18 carbon atoms such as, for example, one of the following:

stearic  
palmitic  
cis-9-octadecenoic acid  
cis,cis-9,12-octadecadienoic acid  
cis,cis,cis-9,12,15-octadecatrienoic acid

in the range of from 1% to 20% by weight, the preferred range being between 3% and 15% by weight. It will be appreciated that the amount of carboxylic fatty acid to be added to the developer formulation to minimize or substantially decrease the frictional forces in the developer system may depend in part on the concentration of organic amine that is employed. It has been found that at the higher concentrations it may be necessary to warm the developer above room temperature to keep the carboxylic acid component in solution.

The following examples of developer solutions which may be employed in accordance with this invention are given for the purpose of illustrating preferred embodiments of the invention. It will be understood, however, that this invention is not limited to these illustrations and embodiments of developer solutions useful in practicing this invention.

It will be appreciated that the combination of an alkanolamine and a carboxylic fatty acid will produce the salt of the alkanolamine. For example, stearic acid will produce the stearate salt of monoethanolamine. All percentages are shown as percent by weight unless otherwise specified.

|  | Example I               | Percent |
|--|-------------------------|---------|
|  | Monoethanolamine        | 60      |
|  | Hexylene glycol         | 20      |
|  | Cis-9-octadecenoic acid | 20      |

The ingredients were mixed together in a mixing vessel until a uniform solution resulted. The solution was charged into the developer trough of a developer unit such as disclosed in copending application Ser. No. 831,685 now U.S. Pat. 3,626,833, which is assigned to the same assignee as the instant invention.

|  | Example II                        | Percent |
|--|-----------------------------------|---------|
|  | Monoethanolamine                  | 60      |
|  | Diethylene glycol monomethylether | 20      |
|  | Diethylene glycol monoethylether  | 17      |
|  | Stearic acid                      | 3       |

|  | Example III                       | Percent |
|--|-----------------------------------|---------|
|  | 2-(2-aminoethoxy)ethanol          | 40      |
|  | Hexylene glycol                   | 25      |
|  | Diethylene glycol                 | 10      |
|  | Diethylene glycol monomethylether | 10      |
|  | Cis,cis-9,12-octadecadienoic acid | 15      |

|  | Example IV                                | Percent |
|--|-------------------------------------------|---------|
|  | Diglycol amine                            | 50      |
|  | Hexylene glycol                           | 25      |
|  | Diethylene glycol monomethylether         | 5       |
|  | Cic,cis,cis-9,12,15-octadecatrienoic acid | 20      |

|  | Example V                     | Percent |
|--|-------------------------------|---------|
|  | Diethanolamine                | 40      |
|  | Diethylene glycol             | 30      |
|  | 4-methoxy-4 methyl-pentanol-2 | 20      |
|  | Palmitic acid                 | 10      |

|  | Example VI              | Percent |
|--|-------------------------|---------|
|  | Morpholine              | 5       |
|  | Monoethanolamine        | 10      |
|  | Dimethylethanolamine    | 5       |
|  | Pentoxol solvent        | 20      |
|  | Cellosolve              | 20      |
|  | Hexylene glycol         | 25      |
|  | Cis-9-octadecenoic acid | 15      |

## Example VII

## Percent

|                                   |    |
|-----------------------------------|----|
| Monoethanolamine                  | 50 |
| N-methylethanolamine              | 10 |
| Triethanolamine                   | 10 |
| Diethylene glycol monomethylether | 10 |
| Cis-9-octadecenoic acid           | 20 |

## Example VIII

## Percent

|                         |    |
|-------------------------|----|
| Monoethanolamine        | 40 |
| Ethylene glycol         | 30 |
| Glycerine               | 10 |
| Water                   | 10 |
| Cis-9-octadecenoic acid | 10 |

## Example IX

## Percent

|                                   |    |
|-----------------------------------|----|
| Monoethanolamine                  | 40 |
| Tetraethylene glycol              | 30 |
| Diethylene glycol monomethylether | 29 |
| Cis,cis-9,12-octadecadienoic acid | 1  |

## Example X

## Percent

|                                   |    |
|-----------------------------------|----|
| Diethylenetriamine                | 50 |
| Diethylene glycol monomethylether | 25 |
| Hexylene glycol                   | 24 |
| Stearic acid                      | 1  |

## Example XI

## Percent

|                         |    |
|-------------------------|----|
| Hexylamine              | 50 |
| Hexylene glycol         | 25 |
| Diethylene glycol       | 15 |
| Cis-9-octadecenoic acid | 10 |

## Example XII

## Percent

|                                   |    |
|-----------------------------------|----|
| Cyclohexylamine                   | 50 |
| Diethylene glycol                 | 25 |
| Diethylene glycol monomethylether | 10 |
| Cis,cis-9,12-octadecadienoic acid | 15 |

## Example XIII

## Percent

|                                   |    |
|-----------------------------------|----|
| Triethanolamine                   | 30 |
| Monoethanolamine                  | 5  |
| Hexylene glycol                   | 5  |
| Diethylene glycol monomethylether | 50 |
| Cis-9-octadecenoic acid           | 10 |

In each of the above developer solutions, the inclusion of the carboxylic fatty acid contributed the necessary lubricity so that the developer apparatus employed resulted in the application of uniform liquid over the area to be developed in the range of from 0.5 to 3 grams per square meter without placing any undue stress on the drive mechanism. The movement of the copy sheet through the developer station was uniform and steady without experiencing any halting or erratic movement as is experienced when using developer liquids without the carboxylic fatty acid producing striations and non-uniform azo-dye formation on the surface of the sheet.

What is claimed is:

1. A developer liquid for developing two-component diazotype material bearing latent images consisting essentially of from 20% to 80% by weight of a liquid organic

amine based on the total developer liquid, said amine being selected from morpholine, piperidine, alkyl morpholine, alkyl piperidine, and the amines of the general formula:



10 wherein  $R_1$  is alkyl, cycloalkyl, alkyl-aryl, alkylo, alkoxy or hydroxyalkoxyalkyl and  $R_2$  and  $R_3$  are alkyl, cycloalkyl, alkyl-aryl, alkyl, alkoxy, hydroxyalkoxyalkyl or hydrogen, wherein  $R_1$  and  $R_2$  and  $R_3$  other than hydrogen are attached to nitrogen through a carbon-nitrogen covalent bond, a carboxylic fatty acid in the range of from 1% to 20% by weight, having a carbon chain length from 16 to 18 carbon atoms, and a polyhydric alcohol, a glycol ether or a monohydric alcohol containing at least 6 carbon atoms.

15 2. A developer composition as claimed in claim 1 wherein the carboxylic fatty acid is oleic acid.

3. The developer composition as claimed in claim 1 wherein the glycol ether is diethylene glycol monomethylether and the carboxylic fatty acid is cis,cis-9,12-octadecadienoic acid.

20 4. The developer composition as claimed in claim 1 wherein the amine has the general formula of



25 30 wherein  $R$  and  $R'$  are the same or different alkyl or hydroxy alkyl radicals or hydrogen,  $X$  is hydrogen, alkyl or hydroxy alkyl, and  $n$  is an integer from 2 to 4, inclusive.

5. The developer composition as defined by claim 4 wherein the amine is an alkanolamine.

35 6. A developer composition as claimed by claim 5 wherein the amine is monoethanolamine.

7. The developer composition as claimed in claim 1 wherein the carboxylic fatty acid is cis,cis,cis-9,12,15-octadecatrienoic acid.

40 8. The developer composition as claimed in claim 1 wherein the carboxylic fatty acid is stearic acid.

9. The developer composition as claimed in claim 1 wherein the carboxylic fatty acid is palmitic acid.

45 10. The developer composition as claimed in claim 1 wherein the amount of carboxylic fatty acid is in the range of from 3% to 15% by weight of the developer liquid.

## References Cited

## UNITED STATES PATENTS

|           |         |                   |         |
|-----------|---------|-------------------|---------|
| 3,130,051 | 4/1964  | Herrick et al.    | 96-49   |
| 2,772,972 | 12/1956 | Herrick et al.    | 96-75 X |
| 3,446,620 | 5/1969  | Parker            | 96-49   |
| 2,807,545 | 9/1957  | Frederick         | 96-75   |
| 3,202,510 | 8/1965  | Hollmann          | 96-49   |
| 2,969,015 | 1/1961  | Klimkowski et al. | 96-49   |
| 2,865,873 | 12/1958 | Hodgins et al.    | 96-49   |
| 3,166,421 | 1/1965  | Gramlich          | 96-49   |
| 3,284,201 | 11/1966 | Meijs et al.      | 96-49   |
| 3,355,295 | 11/1967 | Priest            | 96-49   |
| 3,578,452 | 5/1971  | Parker            | 96-49   |